

1,345,081.

B. K. FORD.  
DUPLEX BOARD.  
APPLICATION FILED JUNE 5, 1919.

Patented June 29, 1920.

*Fig. 1.*



*Fig. 2.*



Inventor

*Ben K. Ford*

By *Pagelum and Spencer*  
*Attorneys*

# UNITED STATES PATENT OFFICE.

BEN K. FORD, OF EAST ORANGE, NEW JERSEY.

## DUPLEX BOARD.

1,345,081.

Specification of Letters Patent. Patented June 29, 1920.

Application filed June 5, 1919. Serial No. 302,010.

To all whom it may concern:

Be it known that I, BEN K. FORD, a citizen of the United States, and residing at East Orange, in the county of Essex and

5 State of New Jersey, have invented a new and Improved Duplex Board, of which the following is a specification.

This invention consists in a two ply board formed of paper of any desired character, 10 one of the plies being given a preliminary coating of a fusible substance such as asphalt, tar, rubber, shellac or resin, which has been permitted to cool and set, one face of the other ply being coated with a cement 15 of any desired character before being brought into contact with the coated face of the first ply, the two coated faces being pressed together to cause the plies to adhere. It also consists in applying finely commi- 20 nuted material such as wood or grain flour, to the fusible coat before it becomes hard, should this fusible material be of such a character that the cement on the second ply will not adhere thereto.

25 In the accompanying drawings, Figure 1 illustrates a duplex board formed of two plies, one of the plies having a fusible coating and the adjacent face of the other being coated with a cement. Fig. 2 is a similar 30 view showing the fusible coat powdered with a substance to which cement will freely adhere.

Similar reference characters refer to like parts throughout the several views.

35 It has been found that when the several plies of paper or straw board containers are secured together by a dissolved cement, such as glue, that the container is not impene- 40 trable to vapors and gases. The minute passages through which the solvent of the cement escapes while the cement is drying permit the escape of moistures in the con- 45 tents of the container. To overcome this difficulty, one of the plies forming such containers is often of duplex board, consisting of two thicknesses of paper secured together by a fused cement, such as asphalt or tar, which penetrates and fills all the minute pas- 50 sages in the board, making it substantially vapor and gas proof.

The objection to this material is that containers cannot be readily produced on spiral tube winding machines of only two thick- 55 nesses as the duplex board must be made up in advance and constitutes one of the two plies.

I have found that I can coat one side of any ordinary fibrous board 1 (Fig. 1) such as is used in making containers with a layer of hot melted asphalt, tar, resin or shellac 60 2 and thus produce a moisture and gas proof sheet which can be employed in the manu- 65 facture of containers. To this thickness I cement a second thickness 3 by means of any desired cement such as ordinary glue 4, the glue being applied to the surface of fused material or to the surface of the other ply which is pressed against the fused material. It is obvious that the first ply may be prepared in great rolls and then slitted pre- 70 paratory to running the strips into a spiral winding machine such as is shown in my prior Patent No. 1,059,046, dated April 15, 1913, and that it or the second ply will be passed through a proper glue applying 75 mechanism before it reaches the winding mandrel. The glue will secure the two plies of the container together in the usual manner.

When the properties of the fusible ma- 80 terial and of the cement are such that they will not adhere, as when one is coated with shellac and the other with ordinary glue, I overcome the difficulty by dusting the surface 5 of the fusible material while still 85 melted with some finely divided substance 6 to which the cement 4 will adhere, pow- 90 dered wood, grain and straw, finely divided cotton fibers and asbestos and neutral earths being suitable for such purpose. 90

It is to be understood that the cement that secures the two plies together is not neces- 95 sarily a dissolved cement, for a fusible cement such as asphalt, gilsonite and petro- lite may be employed, but for ordinary use, glue dissolved in hot water will be found satisfactory.

I claim:

1. A duplex board comprising one layer having one side coated with fused material 100 and a second layer secured to the thus coated side of the first by means of a dis- solved cement.

2. A fibrous material having one side coated with fused material whose surface is 105 impregnated with finely divided material to which cement readily adheres and a sheet of fibrous material secured by a dissolved cement to the fused material and to the material with which the surface of said 110 fused material is impregnated.

3. A fibrous material having one side

coated with fused material whose surface is impregnated with finely divided wood and a sheet of fibrous material secured by a dissolved cement to the fused material and 5 to the material with which the surface of said fused material is impregnated.

4. A duplex board comprising one ply having one side coated with fused material whose surface is impregnated with finely 10 divided material to which cement readily adheres and a second ply secured to the thus coated side of the first ply by means of glue.

5. A duplex board comprising one layer having one side coated with fused material and a second layer secured to the thus coated 15 side of the first by means of a dissolved cement, the fused material being intermingled with the cement by having fine particles extending into the capillary passages in the cement and in the second layer of the du- 20 plex board through which the solvent of the cement has escaped.

BEN K. FORD.